

# UNITED STATES PATENT OFFICE.

WILLIAM AUGUSTUS HALL, OF NEW YORK, N. Y., ASSIGNOR TO AMERICAN MAHOGANY COMPANY, A CORPORATION OF MAINE.

## VULCANIZING AND COLORING WOOD.

No. 891,987.

Specification of Letters Patent.

Patented June 30, 1908.

Application filed May 13, 1907. Serial No. 373,230.

To all whom it may concern:

Be it known that I, WILLIAM AUGUSTUS HALL, a citizen of the United States, residing at New York, in the county of New York and State of New York, have invented or discovered certain new and useful Improvements in the Art of Vulcanizing and Coloring Wood, of which the following is a specification.

This invention relates to the art of treating wood for the purpose of vulcanizing or hardening and coloring the same, so that products resembling some of the higher priced woods, and produced from some of the more common or cheaper woods, will result.

Attempts have heretofore been made to darken some of the cheaper woods, such as maple and white and yellow birch, for the purpose of making them resemble some of the higher priced woods, such as black cherry and black walnut, by boiling the woods in closed receptacles under pressure resulting in temperatures considerably above 212° F. This boiling of the wood in water or other liquids at temperatures approximating 230° F., or above, changes the chemical and physical properties of the wood, so that, in drying, it has a tendency to twist and check or crack. Moreover such boiling process takes out more or less of what is known in the wood-working trade as the "life" of the wood, and renders the same brittle and much less elastic than in its natural state; and the present invention or discovery has for its object to obviate these objections so that the wood may be vulcanized or hardened and also colored, and at the same time be rendered tougher than in its first or normal condition, instead of becoming more brittle. This object is accomplished by adding a suitable alkali or alkalies, such as ammonium hydroxid or sodium hydroxid, to the water in which the wood is boiled, thereby producing weak alkaline solutions which act upon the wood and render it tougher than it was before the treatment, the hot alkaline solution also coloring the wood a rich brown. This hardening and toughening effect is due presumably to two causes; first, to a semi-solution of the ligneous matter in the wood, forming an adhesive, gummy mass which more closely binds together the cellulose structure of the wood; and, second, to the hydrolytic action of the alkali or alkalies on the lignin-cellulose composition, similar to the action known as mer-

I have discovered that woods which are penetrated with solutions of ammonium hydroxid and then boiled at temperatures exceeding 212° F., become very much tougher and harder than the natural woods, but have a greater tendency to warp and check or crack than the woods which have been simply boiled in water, and the woods thus boiled in the ammonium hydroxid solution are rendered very much darker in shade than when simply boiled in water, particularly in the heart portions of the wood. I have also discovered that woods treated with sodium hydroxid have become as hard and tough, and even more so, as those treated with ammonium hydroxid, but with much less tendency to warp or twist and crack or check; but it has been found that it is well nigh impossible to thoroughly permeate the wood treated with the sodium hydroxid solution, even by the best of vacuum and pressure processes; presumably for the reason that a gelatinizing occurs on or near the surface of the wood which largely prevents further penetration of the sodium hydroxid solution into the wood; so that the sodium hydroxid solution produces, when the wood is dried, what may be termed "case hardening" on the outer parts of the wood, without vulcanizing and coloring the wood throughout. While, from one point of view, the sodium hydroxid solution is more desirable than the ammonium hydroxid solution, in that it better toughens and hardens the wood and leaves it with much less tendency to warp, twist and check or crack, it is much less desirable from another point of view, in that it is practically impossible to permeate the wood throughout with the sodium hydroxid solution. I have discovered, however, that a mixture of sodium and ammonium hydroxids results in a solution with excellent penetrating qualities; and that the presence of the sodium hydroxid prevents, to a great extent, the checking and warping tendencies of the ammonium hydroxid. It is by this combination of the two hydroxids that I obtain the good effects of each without the ill effects of either, and am able to color the wood to the fine rich brown shades produced by ammonia, and at the same time avoid the astringent characteristics of the ammonia which cause undue shrinking when the wood is dried, and which produce the warping and checking tendencies referred to; and in this

mixed solution the ammonium hydroxid lessens the extreme hydrolytic action of the sodium hydroxid and enables the solution to completely penetrate the wood.

5 The solution which I find to produce the best results in the treatment of the wood for the purpose of vulcanizing and coloring the same, as above referred to, comprises, in its most desirable proportions, about 3 lbs. of 10 sodium hydroxid to 2 gals. 26% ammonium hydroxid and 50 gals. of water.

In carrying the invention into effect the wood is first thoroughly dried and is then preferably subjected to the action of a 5 vacuum in a closed receptacle of above 25 inches of mercury, for the purpose of removing the air from the wood and rendering it absorbent. The alkaline solution, preferably comprising the ingredients in the 20 proportion just above mentioned, is then drawn or forced into the receptacle and a high hydraulic or other pressure is then preferably applied to force the alkaline solution into and throughout the body of the wood, although 25 this pressure is not really necessary unless the wood being treated is more than  $\frac{1}{4}$  of an inch in thickness, but if the wood be an inch or more in thickness it is absolutely necessary, in order that the wood may be penetrated 30 throughout by the alkaline solution. The wood is boiled for several hours (the time varying according to the thickness of the wood) in a closed receptacle either before or after the hydraulic pressure is applied, but 35 preferably afterwards.

By practicing the invention or discovery, as above described, very tough and hard products of artificially colored wood, with rich brown shades, will be produced. Although, in the practice of the invention or discovery, an alkaline solution comprising sodium and ammonium hydroxids is preferably employed, the invention or discovery is not to be understood as being limited to these 45 particular alkalies or hydroxids; as potassium hydroxid and some other alkaline salts

might be used, with good effect, in place of the sodium hydroxid, to lessen the tendency of the wood to warp and check. So far, however, as has yet been demonstrated, by the practice of the invention or discovery, the alkaline solution comprising sodium and ammonium hydroxids in about the proportion above stated produces the best results.

Having thus described my invention or discovery, I claim and desire to secure by Letters Patent:—

1. The herein described improvement in the art of vulcanizing and coloring wood, consisting in boiling the same in a closed receptacle in an alkaline solution comprising a mixture of sodium and ammonium hydroxids, in substantially the proportions stated.

2. The herein described process of treating wood, for the purpose of coloring and vulcanizing the same, consisting in first thoroughly drying the wood, then subjecting the dried wood, in a closed receptacle, to the action of a vacuum for the purpose of removing the air therefrom and rendering the same absorbent, and subsequently forcing an alkaline solution into and throughout the wood, by high pressure, and boiling the wood in said solution.

3. The herein described process of treating wood for the purpose of coloring and vulcanizing the same, consisting in first thoroughly drying the wood, then subjecting the dried wood, in a closed receptacle, to the action of a vacuum, for the purpose of removing the air therefrom and rendering the same absorbent, and subsequently forcing an alkaline solution, consisting of a mixture of sodium and ammonium hydroxids, into and throughout the body of the wood, by high pressure, and boiling the wood in said solution.

In testimony whereof I affix my signature, in presence of two witnesses.

WILLIAM AUGUSTUS HALL.

Witnesses:

JOHN C. McCUSKER,  
C. M. SWEENEY.